

# United States Patent

[19]

Shirasu et al.

[11] 3,775,124

[45] Nov. 27, 1973

[54] STABILIZING METHOD AND  
COMPOSITION FOR COLOR  
PHOTOGRAPHIC PROCESSING

[75] Inventors: Kazuo Shirasu; Mitsuo Ozawa;  
Yasuhide Ogawa, all of Kanagawa,  
Japan

[73] Assignee: Fuji Photo Film Co., Ltd.,  
Kanagawa, Japan

[22] Filed: June 14, 1972

[21] Appl. No.: 262,896

[30] Foreign Application Priority Data

June 14, 1971 Japan..... 46/42385

[52] U.S. Cl..... 96/56, 96/61, 96/66.4,  
96/109

[51] Int. Cl..... G03c 7/00

[58] Field of Search..... 96/56, 66.4, 109,  
96/61

[56]

## References Cited

### UNITED STATES PATENTS

|           |         |                     |         |
|-----------|---------|---------------------|---------|
| 2,017,295 | 10/1935 | Schultes et al..... | 96/66.4 |
| 3,236,652 | 2/1966  | Kennard et al. .... | 96/56   |
| 3,457,079 | 7/1969  | Koda et al. ....    | 96/109  |

Primary Examiner—Norman G. Torchin  
Assistant Examiner—Richard L. Schilling  
Attorney—Richard C. Sughrue et al.

[57]

## ABSTRACT

A stable processing solution for improving the stability of color images of color photographic materials is disclosed. The processing solution contains pyrogallol-1,3-dimethyl ether.

8 Claims, No Drawings

## STABILIZING METHOD AND COMPOSITION FOR COLOR PHOTOGRAPHIC PROCESSING

### BACKGROUND OF THE INVENTION

#### 1. Field of the Invention

This invention relates to a processing composition for improving the stability of images of color photographic materials and having improved stability of itself.

More particularly, the invention relates to a stabilized processing composition containing pyrogallol-1,3-dimethyl ether for improving the stability of color images of color photographic materials by processing the color photographic materials having the color images with the composition.

#### 2. Description of the Prior Art

In general, it is well known that color photographs having color images of dyes such as indophenol, indamine, indoaniline, and azomethine formed from an aromatic amine developer and couplers are inferior in light fastness. It is also known that the light fastness of those color photographs can be increased using the following methods;

1. A compound absorbing ultraviolet light can be incorporated in the color photographic materials (See, e.g., the specifications of U.S. Pat. Nos. 2,632,701 and 2,747,996).

2. A reducing agent or an antioxidant can be incorporated in the color photographic materials (See, e.g., the specifications of U.S. Pat. Nos. 2,384,658 and 3,095,302).

For incorporating those compounds in the color photographic materials, they can be preliminary incorporated in the emulsion layers of the color photographic materials or they can be introduced into the emulsion layers of the color photographic materials during processing of the materials. Those methods may be alternatively employed depending upon the nature of each compound to be incorporated or the characteristics of the photographic sensitive materials.

A color photographic sensitive material is generally subjected to a series of the following processing steps: For example, to the steps of color development, stop fixing, water washing, bleaching, water washing, hardening fixing, water washing, and stabilization as described in *The British Journal of Photography*, September 27, 838(1968); to the steps of pre-bath processing, rinsing, color development, fixing, water washing, bleaching, water washing, fixing, water washing, and stabilization as described in *Journal of the S.M. P. T. E.*, Vol. 61, No. 12, 667(1963); or to the steps of color development, blixing, water washing, and stabilization as described in the specification of German Pat. No. 1,928,554.

It is known to use a processing bath containing a compound having a hydroxyl group, an amino group, or a substituted amino group for improving the stability of color images in the color photographic processes referred to above (See, e.g., the specification of U.S. Pat. No. 2,384,658). However, the color photographic material processed by a bath containing hydroquinone or a derivative thereof as described in the German Patent specification has the disadvantage that markedly brown stains form on the non image-bearing portions of the color photographic material by light exposure although the light fastness of the magenta dye itself may be improved. Also, when a color photographic material is processed with a bath containing ascorbic acid as de-

scribed in the above German Patent specification, the light fastness of the magenta dye itself may be improved as in the above case, but the color photographic material processed suffers the formation of brown stains and further the cyan density is reduced greatly.

Similarly, it is known that gallic acid improves the stability of images (See, e.g., the specification of U.S. Pat. No. 3,069,262). However, in addition to the fact that the effect of the compound for improving the light fastness of the magenta dye is slight as compared with the compound previously referred to, brown stains form greatly.

### SUMMARY OF THE INVENTION

15 As the result of the inventors' various investigations for improving these disadvantages, it has been discovered that by processing a color photographic material subjected to conventional processings in an aqueous solution containing pyrogallol-1,3-dimethyl ether, the light fastness of not only the magenta dye but also the yellow dye is remarkably improved without being accompanied by the formation of brown stains at the non-image bearing portions by light exposure. Moreover, it has also been discovered that by processing with the compound in this invention, the discoloration and fading of the cyan dye due to heat and also the fading of the yellow dye due to humidity are prevented.

### DETAILED DESCRIPTION OF THE INVENTION

30 An object of the invention is, therefore, to provide a processing composition for preventing the color images of color photographic material from being faded by the actions of light, humidity, or heat.

Another object of this invention is to provide a color photographic material such as a color film, a color transparency, and a color print stable to light or heat by processing the color photographic material with a stabilizing bath containing a specific compound.

40 Furthermore, the compound in the present invention can be effectively used in an aqueous solution containing at least one of urea, guanidine, and water-soluble derivatives of these materials as described in the specification of U.S. Application Ser. No. 110,291, filed Jan. 27, 1971, and di- or tri-hydroxybenzene or derivative thereof. Still further, the compound of this invention can be effectively used together with a phenolic compound described in the specification of U.S. application Ser. No. 182,558, filed Sept. 21, 1971.

45 It is generally known that when photographic sensitive materials and processing solutions are placed under certain conditions, microorganisms grow therein. Since in the former case the microorganisms grow mainly in the protective colloid such as gelatin of the photographic sensitive material, the image portions are attacked by such microorganisms. That is to say, red or purple spot-like foreign substances are formed in an early period and when the spots grow, the image portions become unobservable and finally are bleached. Such a disadvantage is quite undesirable from the standpoint of the preservation of photosensitive materials. In the latter case, colloid foreign substances are formed in the processing solutions and they emit bad smells. As this condition progresses, the intensity of the bad smell increases and the processing solutions lose their desired properties.

50 It is known that the growth of the microorganisms as previously indicated is observed when photographic

sensitive materials are stored under such high temperature and high humidity conditions as are suitable for the growth thereof, for instance at temperatures of 30°-40° C and relative humidities of 70-90% RH. As a means for preventing the growth of microorganisms in photographic sensitive materials, a pentachlorophenol (sodium salt) containing bath and an Ansco 955 stabilization rinse bath as shown in *Photographic Science and Engineering*, Vol. 3, No. 3, (1959) are known. Also, it is known that a hydantoin derivative prevents the growth of microorganisms in photographic sensitive materials as described in, e.g., the specification of U.S. Pat. No. 2,762,768.

However, although those compound referred to above may be effective for preventing the growth of microorganisms in photographic sensitive materials, they are hardly or less effective for processing compositions of solutions when they are incorporated in the processing compositions or solutions.

On the other hand, it is also known that when a processing composition for photographic materials is preserved for a long period of time at high temperatures of, e.g., 20°-45°C., microorganisms grow in the processing composition. As a method of preventing such a growth of microorganisms in the processing composition, it is known to incorporate therein a nitroalcohol derivative as described in the specification of U.S. Pat. No. 3,542,553. However, the incorporation of the nitroalcohol derivative in a processing composition for photographic sensitive materials may be effective for preventing the growth of microorganisms in the processing composition but is hardly effective for preventing the growth of microorganisms in the photographic materials processed in such a processing composition containing the derivative. Furthermore, the photographic sensitive materials processed in a bath containing the nitroalcohol derivative also suffer the formation of brown stains due to the action of light or heat.

The inventors have also investigated various compounds which are effective for preventing the growth of microorganisms in processing compositions and simultaneously in photographic materials processed by the compounds without adverse influences on either of them, and as the results thereof it has been discovered that the above purpose also can be attained by using pyrogallol-1,3-dimethyl ether.

Another object of this invention is, therefore, to provide a means to prevent the growth of microorganisms in a processing composition for photographic sensitive materials unaccompanied by adverse influences on the function of the processing composition and at the same time to prevent also the growth of microorganisms in the photographic sensitive materials processed by the composition without giving rise to any adverse influences on the photographic sensitive materials.

The advantages of using the processing composition of this invention containing pyrogallol-1,3-dimethyl ether are as indicated below.

1. The light fastness of the yellow dye of a color photographic material to various lights is improved by processing the color photographic material with the processing composition.

2. The light fastness of the magenta dye of a color photographic material to various lights is improved.

3. The processing of a color photographic sensitive material with the processing composition prevents the discoloring and fading of the cyan dye thereof due to

the action of heat and also the formation of color stains therein due to the action of heat.

4. The processing of a color photographic sensitive material with the processing composition prevents the fading of the yellow dye thereof due to the action of humidity. 5. Microorganisms do not grow in the processing composition.

6. The processing of photographic sensitive material prevents the growth of microorganisms in the photographic sensitive material.

It is preferable to use the compound of this invention together with di- or polyethylene glycol because in such a case the rate of dissolution of the compound in water can be increased.

A suitable amount of pyrogallol-1,3-dimethyl ether which can be used in the processing composition of this invention generally ranges from 0.1 to 10 g/liter preferably from about 1 to 3 g/liter. The present invention can be used instead of the processing bath described in *The British Journal of Photography*, September 27, 839(1968), the process bath described in *Journal of the S. M. P. T. E.* Vol. 61, No. 12, 682(1963), and the processing composition described in the specification of U.S. Pat. No. 3,582,322 without any limitations but the compound of this invention is more effectively used when incorporated in a stabilization bath. Furthermore, the compound of this invention is more effectively incorporated in the stabilization bath described in the specification of U.S. application Ser. No. 21,184, filed Mar. 19, 1970.

Now, suitable examples of the photosensitive materials which can be processed effectively by the processing composition of this invention are color photographic sensitive materials containing the acetonilide yellow couplers described in the specification of U.S. Pat. No. 3,551,156, the pyrazolone magenta couplers described in the specification of U.S. Pat. No. 3,558,319, or the specification of U.S. Pat. No. 3,337,344, and the phenolic couplers described in the specifications of U.S. Pat. Nos. 2,423,703 and 2,474,293 but the photographic sensitive materials to be processed by the processing composition of this invention are not limited to only the above-described color photographic sensitive materials.

Furthermore, the processing composition of this invention can be more effectively applied to the photographic sensitive materials containing a ultraviolet absorbent as described in, e.g., the specification of U.S. Pat. No. 3,352,681 and the specification of U.S. Pat. No. 3,253,921.

Typical experimental results on the stability of the images of the photographic sensitive materials processed by the processing bath of this invention and typical experimental results on the preservative property of the processing composition of this invention will be described by reference to the following examples but the invention is not to be interpreted as limited to these examples.

#### EXAMPLE 1

|    | Color Developing Solution             | (pH 10.6) |
|----|---------------------------------------|-----------|
| 60 | Sodium Metaborate                     | 25.0 g    |
|    | Sodium Sulfite                        | 2.0 g     |
|    | Hydroxylamine Sulfate                 | 2.0 g     |
|    | Potassium Bromide                     | 0.5 g     |
| 65 | 6-Nitrobenzimidazole Nitrate          | 0.02 g    |
|    | Sodium Hydroxide                      | 4.0 g     |
|    | Benzyl Alcohol                        | 15.8 ml   |
|    | Diethylene Glycol                     | 20.0 ml   |
|    | N-Ethyl-N-β-(methanesulfonamidoethyl- |           |

|                           |          |
|---------------------------|----------|
| p-phenylenediamine)       | 8.0g     |
| Water added to make       | 1 liter  |
| Stop Fixing Solution      |          |
| Ammonium Thiosulfate      | 120.0 g  |
| Sodium Pyrosulfite        | 20.0 g   |
| Glacial Acetic Acid       | 10.0 g   |
| Water added to make       | 1 liter  |
| Bleaching Solution        | (pH 7.2) |
| Potassium Nitrate         | 25.0 g   |
| Ferricyanide              | 20.0 g   |
| Potassium Bromide         | 8.0 g    |
| Boric Acid                | 5.0 g    |
| Borax                     | 2.5 g    |
| Water added to make       | 1 liter  |
| Hardening Fixing Solution | (pH 9.5) |
| Ammonium Thiosulfate      | 120.0 g  |
| Sodium Sulfite            | 5.0 g    |
| Formalin (35-40%)         | 2.5 g    |
| Water added to make       | 1 liter  |

A color photographic paper prepared by applying successively to a baryta-coated paper a blue-sensitive silver iodobromide emulsion layer containing a yellow coupler, benzoylaceto-2-chloro-5-decylloxycarbonyl anilide, an intermediate gelatin layer, a green-sensitive silver chlorobromide emulsion layer containing a magenta coupler, 1-phenyl-3-[3-(N-butylcaprylamidopropionamido)]-5-pyrazolone, an intermediate gelatin layer, a red-sensitive silver silver chlorobromide emulsion layer containing a cyan coupler, 1-hydroxy-2-[3-(2,4-t-amylphenoxy)propyl]naphthamide, and a protective gelatin layer in this order was subjected to the following processings successively at 30°C using the processing solutions having the above-indicated compositions.

That is to say, the color photographic paper was, after imagewise exposure, subjected to a color development for 7 minutes, a stop fixing for 2 minutes, a water washing for 2 minutes, a bleaching for 2 minutes, a water washing for 2 minutes, a hardening fixing for 2 minutes, and then a water washing for 4 minutes.

Thereafter, the color photographic paper thus processed was further processed for 2 minutes at 30.0°C in one of the processing baths A-F having the compositions shown in the following table.

| Compound                                  | Bath  |       |       |       |       |       |
|-------------------------------------------|-------|-------|-------|-------|-------|-------|
|                                           | A     | B     | C     | D     | E     | F     |
| Tartaric acid, g-----                     | 10.0  | 10.0  | 10.0  | 10.0  | 10.0  | 10.0  |
| Zinc sulfate, g-----                      | 10.0  | 10.0  | 10.0  | 10.0  | 10.0  | 10.0  |
| Sodium metaborate, g-----                 | 20.0  | 20.0  | 20.0  | 20.0  | 20.0  | 20.0  |
| Pyrogallol-1,3-dimethyl ether, g-----     | 3.0   | ----- | 3.0   | 3.0   | 3.0   | 3.0   |
| p-Methoxy hydroquinone, g-----            | ----- | 2.0   | ----- | ----- | ----- | ----- |
| Urea, g-----                              | ----- | ----- | 30.0  | ----- | ----- | ----- |
| Hydroquinone, g-----                      | ----- | ----- | 2.0   | ----- | ----- | ----- |
| Pyrogallol, g-----                        | ----- | 3.0   | ----- | ----- | ----- | ----- |
| Gallic acid, g-----                       | ----- | ----- | 3.0   | ----- | ----- | ----- |
| Water added to make 1 liter in all cases. | 5.0   | 5.0   | 5.0   | 5.0   | 5.0   | 5.0   |
| pH-----                                   | 5.0   | 5.0   | 5.0   | 5.0   | 5.0   | 5.0   |

The samples processed in the above processing bath were tested with respect to the stability of the image by exposing them to a fluorescent lamp of 10,000 lux. The faded percentage after an exposure of 10 days is shown in the following table.

| Processing Bath | Faded Percentage* |         |      |       |
|-----------------|-------------------|---------|------|-------|
|                 | Yellow            | Magenta | Cyan | ΔDy   |
| A               | 27%               | 45%     | 10%  | +0.07 |
| B               | 15%               | 15%     | 10%  | +0.07 |
| C               | 28%               | 30%     | 10%  | +0.15 |
| D               | 27%               | 44%     | 10%  | +0.16 |
| E               | 14%               | 10%     | 10%  | +0.08 |
| F               | 11%               | 11%     | 10%  | +0.06 |

Also, the color photographic papers processed in the above-indicated processing baths were tested with respect to the stability of the image by exposing them directly to sun light. The faded percentage of the color

images after an exposure of 12 days is shown in the following table.

| Processing Bath | Faded Percentage* |         |      |       |
|-----------------|-------------------|---------|------|-------|
|                 | Yellow            | Magenta | Cyan | ΔDy   |
| A               | 30%               | 44%     | 13%  | +0.07 |
| B               | 16%               | 15%     | 13%  | +0.07 |
| C               | 28%               | 29%     | 13%  | +0.15 |
| D               | 27%               | 42%     | 13%  | +0.16 |
| E               | 15%               | 11%     | 13%  | +0.08 |
| F               | 12%               | 12%     | 13%  | +0.06 |

10 The faded percentage\* is the ratio of the color density of the portion having an initial color density of 1.0 reduced during the test. The ΔDy is the density increase of the non-exposed portions expressed by the density of yellow component.

15 The experimental results show clearly the following:

1. The processing bath C containing a known compound similar to the compound in the present invention had the effect of preventing the fading of the magenta image by light in comparison with the conventional processing bath A but was ineffective as to yellow images and additionally was accompanied by the formation of a great amount of brown stains. Also, the processing bath D showed no fading preventing effect of the color images and further showed a great increase in the formation of brown stains.

2. The processing bath B of this invention showed a remarkable fading prevention effect of the magenta images due to light and a remarkable fading preventing effect of yellow images by light. Also, in this case, no increase of stains due to light exposure was observed.

3. The processing baths E and F containing the compound in the present invention and the above-indicated known compounds were more effective than the processing bath B.

35 Then, the samples processed in the processing baths shown above were stored for 7 days at 76.7°C and under a low humidity. In this case the ratio of the color density of the portion having an initial color density of 1.0 reduced during the test and the density (ΔDy) of 40 the stain increase at the non-exposed portions is shown in the following table.

| Processing Bath | Faded Percentage |         |      |       |
|-----------------|------------------|---------|------|-------|
|                 | Yellow           | Magenta | Cyan | ΔDy   |
| A               | 0                | 2%      | 15%  | +0.06 |
| B               | 0                | 1%      | 8%   | +0.06 |
| C               | 0                | 2%      | 14%  | +0.12 |
| D               | 0                | 2%      | 15%  | +0.13 |
| E               | 0                | 2%      | 8%   | +0.06 |
| F               | 0                | 5%      | 7%   | +0.05 |

Furthermore, the samples processed above were also stored for 14 days at 40°C under a relative humidity of 90% RH and the results obtained are shown in the following table.

| Processing Bath | Faded Percentage |         |      |       |
|-----------------|------------------|---------|------|-------|
|                 | Yellow           | Magenta | Cyan | ΔDy   |
| A               | 11%              | 2%      | 3%   | +0.03 |
| B               | 5%               | 2%      | 2%   | +0.02 |
| C               | 10%              | 1%      | 3%   | +0.04 |
| D               | 11%              | 2%      | 3%   | +0.04 |
| E               | 5%               | 2%      | 2%   | +0.03 |

55 60 From these experimental results it is clear that the samples processed by using the processing baths of this invention was improved in the stability of the cyan image to heat and also were improved in the stability of the yellow image to humidity.

65 Also, when the same experiments as above were conducted using color photographic films in place of the above color photographic paper, almost the same results were obtained.

## EXAMPLE 2

A color photographic positive film prepared by applying to cellulose acetate film a blue-sensitive silver iodobromide emulsion layer containing a yellow coupler, an intermediate gelatin layer, a red-sensitive silver chlorobromide emulsion layer containing a cyan coupler, an intermediate gelatin layer, a green-sensitive silver chlorobromide emulsion layer containing a magenta coupler, and a intermediate gelatin layer successively in this order was subjected to the following processings at 21°C. The couplers used in the color positive film were same as those used in Example 1.

The color positive film was, after image-wise exposure, subjected to the steps of pre-treatment for 10 seconds, rinse for 15 seconds, development for 12 minutes, rinse for 15 seconds, fixing for 4 minutes, water washing for 4 minutes, bleaching for 8 minutes, fixing for 4 minutes, and water washing for 8 minutes.

The compositions of the processing solution used in the above processings were as follows.

| Developing Solution                          | (pH 10.65) | 2.0 g ti (produced by |
|----------------------------------------------|------------|-----------------------|
| Calgon*                                      |            |                       |
| (Calgon, Inc.)                               |            |                       |
| Sodium Sulfite                               | 4.0 g      | 25                    |
| N,N-Diethyl-p-phenylenediamine Hydrochloride | 3.0 g      |                       |
| Sodium Carbonate Monohydrate                 | 20.0 g     |                       |
| Potassium Bromide                            | 2.0 g      |                       |
| Water added to make                          | 1 liter    |                       |

\*Trade name of sodium polymetaphosphate,  $(NaPO_3)_x$  comprising 32.1% by weight  $Na_2O$ , 66.8% by weight  $P_2O_5$ , 0.2% by weight  $Na_2SO_4$  and 0.1% by weight  $NaCl$ .

The pre-treatment bath contained sodium hydroxide, the fixing bath contained sodium thiosulfate, and the bleaching bath contained potassium bichromate.

Thereafter, the color photographic film thus processed was further processed for 2 minutes in a processing bath containing the compound shown in the following table and dried.

| Processing Bath | Compound in the Bath          | Amount    |
|-----------------|-------------------------------|-----------|
| G               | Pyrogallol-1,3-dimethyl ether | 2 g/liter |
| H               | Pyrogallol                    | 2 g/liter |
| I               | Hydroquinone                  | 2 g/liter |
| J               | Gallie Acid                   | 2 g/liter |
| K               | 2,3-Dihydroxybenzoic Acid     | 2 g/liter |
| L               | Ascorbic Acid                 | 2 g/liter |

The samples processed in each of the above processing baths were exposed for 50 hours to a xenon lamp of about 100,000 lux and then the ratio of the color density of the portion having an initial color density of 1.0 reduced during the test and the stain increase density ( $\Delta Dy$ ) of the non-exposed portion are shown in the following table. The xenon lamp used in the experiment was a light source having very similar spectral distribution and intensity to the day light energy of sun light.

| Processing Bath | Yellow | Magenta | Cyan | $\Delta Dy$ |
|-----------------|--------|---------|------|-------------|
| G               | 9%     | 8%      | 12%  | +0.06       |
| H               | 20%    | 20%     | 13%  | +0.12       |
| I               | 19%    | 17%     | 12%  | +0.10       |
| J               | 20%    | 30%     | 13%  | +0.12       |
| K               | 20%    | 28%     | 13%  | +0.11       |
| L               | 20%    | 22%     | 15%  | +0.25       |
| M               | 20%    | 22%     | 15%  | +0.05       |
| None            | 20%    | 30%     | 13%  | +0.05       |

From the experimental results shown above, it is clear that the processing baths H, I, and L each containing the known compound had a fading prevention

effect of magenta images due to light but were ineffective for the fading prevention of yellow images and further in this case the formation of color stains increased remarkably. Further, the processing baths J and K showed almost no fading prevention effect to color images and also in these cases a remarkable increase of brown stains was observed.

On the other hand, the processing bath G of the present invention showed a remarkable fading prevention effect of magenta images due to light and also a remarkable fading prevention effect of yellow images due to light and also in this case the increase of the formation of color stains due to the action of light was hardly increased.

Furthermore, when the samples were processed in each of the processing solutions shown above for 7 days at 76.7°C under a low humidity condition or for 14 days at 40°C under a relative humidity of 90 percent, it was confirmed that the sample processed using the processing solution of this invention had a cyan image stable to heat and also yellow image stable to humidity. On the other hand, when the processing baths containing conventional compounds were used, the stability of the color images of the color photographic film was not improved and further remarkable brown stains formed.

Also, when the same procedure as above was conducted using a color photographic paper in place of the color positive film, almost the same results were obtained.

## EXAMPLE 3

A color photographic paper prepared in the same way as described in Example 1 was subjected to the following processing steps as 29.5°C.

The color photographic paper was, after image-wise exposure, subjected to the steps of development for 6 minutes, blixing for 2 minutes, and water washing for 4 minutes in this order. The composition of the developing solution used above was the same as that of the developing solution used in Example 1, while the blixing solution had the following composition:

Ethylenediamine Tetraacetic Acid Iron Salt — 45 g  
Ammonium Thiocyanate — 10 g  
Sodium Sulfite — 10 g  
Ammonium Thiosulfate (60%) — 100 ml  
Ethylenediamine Tetraacetic Acid 4-Sodium Salt — 5 g  
Water added to make — 1 liter

Thereafter the sample thus processed was further processed for 2 minutes in each of the processing baths having the compositions shown in the following table, rinsed for 15 seconds, and then dried.

| Compound                                      | Bath |      |      |      |      |
|-----------------------------------------------|------|------|------|------|------|
|                                               | M    | N    | O    | P    | Q    |
| Potassium alum, g.                            | 30.0 | 30.0 | 30.0 | 30.0 | 30.0 |
| Sodium citrate, g.                            | 5.0  | 5.0  | 5.0  | 5.0  | 5.0  |
| Boric acid, g.                                | 5.0  | 5.0  | 5.0  | 5.0  | 5.0  |
| Sodium metaborate, g.                         | 4.5  | 4.5  | 4.5  | 4.5  | 4.5  |
| Pyrogallol-1,3-dimethyl ether, g.             | 2.5  |      |      | 2.5  | 2.5  |
| p-Methoxy hydroquinone, g.                    |      |      |      | 2.0  |      |
| Urea, g.                                      |      |      |      |      | 30.0 |
| Hydroquinone, g.                              |      |      | 3.0  |      | 2.0  |
| Pyrogallol, g.                                |      |      |      | 3.0  |      |
| Gallie acid, g.                               |      |      |      |      | 3.0  |
| Water added to make 1 liter in all the cases. |      |      |      |      |      |
| pH                                            | 3.5  | 3.5  | 3.5  | 3.5  | 3.5  |

The samples processed in each of the processing baths were exposed to a fluorescent lamp of 10,000 lux for 10 days.

The ratio of the color density of the portion having an initial color density of 1.0 reduced during the test and the density of the stain increase at the unexposed portions in this case are shown in the following table.

| Processing Bath | Faded Percentage |         |      |       |
|-----------------|------------------|---------|------|-------|
|                 | Yellow           | Magenta | Cyan | ΔDy   |
| M               | 30%              | 40%     | 10%  | +0.02 |
| N               | 16%              | 13%     | 10%  | +0.02 |
| O               | 31%              | 27%     | 10%  | +0.11 |
| P               | 30%              | 40%     | 10%  | +0.12 |
| Q               | 15%              | 9%      | 10%  | +0.03 |
| R               | 12%              | 10%     | 10%  | +0.01 |

From these experimental results, it is clear that the processing bath O containing the conventional compound similar to the compound of this invention gave a fading prevention effect of magenta images due to light in comparison with the conventional processing bath M but it was ineffective for the fading prevention of yellow images and further in the case of processing in the processing bath O, a remarkable increase of the formation of brown stains was observed. Furthermore, the conventional processing bath P gave no fading prevention effect to color images and in this case, a remarkable increase in the formation of yellow stains was observed. On the other hand, the processing bath N of this invention showed a more remarkable fading prevention effect of the magenta images due to light and a remarkable fading prevention effect of the yellow images due to light. In this case, an increase of color stains was hardly observed. Moreover, the processing baths Q and R each containing the compound of this invention together with the conventional compound were found to be more effective than the processing bath N.

On the other hand, when the samples processed in each of the above-described processing baths were stored for 7 days at 76.7°C. under a low humidity condition or for 14 days at 40°C under a relative humidity of 90% RH, the sample processed in the processing bath of this invention showed an improved stability of the cyan images to heat and also an improved stability of the yellow images to humidity. On the other hand, when the processing bath containing the conventional compound was employed, the stability of the color images of the samples was not improved and further remarkable color stains formed.

#### EXAMPLE 4

A color photographic positive film was prepared according to the method as described in Example 2 and was subjected to the processing steps of pre-treatment for 10 seconds, rinse for 15 seconds, development for 12 minutes, rinse of 15 seconds, fixing for 4 minutes, water washing for 4 minutes, bleaching for 8 minutes, water washing for 8 minutes, fixing for 4 minutes, and water washing for 8 minutes using the same procedures as in Example 2.

Thereafter, the color positive film thus processed was further processed in a processing bath having the following composition for 2 minutes and dried.

| Processing Bath | Compound in the Bath          | Amount      |
|-----------------|-------------------------------|-------------|
| S               | Monomethylol Hydantoin        | 0.2 g/liter |
| T               | Pentachlorophenol Sodium salt | 1.0 g/liter |
| U               | 2-Nitro-1,3-propanediol       | 0.1 g/liter |
| V               | pyrogallol-1,3<br>Ether       | 1.0 g/liter |

When each sample thus processed in the above processing bath was stored at 25°C and a relative humidity of 90% RH, the condition of microorganism growth in the sample was observed, the results of which are shown in the following table.

| Bath | Days:  |         |         |         |         |
|------|--------|---------|---------|---------|---------|
|      | 7 days | 14 days | 21 days | 28 days | 56 days |
| S    | 0      | 0       | 0       | 30      | +++     |
| T    | 0      | 0       | 0       | +       | +++     |
| U    | 0      | 0       | +       | ++      | +++     |
| V    | 0      | 0       | 0       | 0       | 0       |
| None | 0      | +       | ++      | +++     | ++0     |

In the above table, (0) means that no microorganism growth was observed (+) means that microorganisms grew slightly (1-2 spots); (++) means that microorganisms grew considerably (5-6 spots); and (+++) means that microorganisms grew throughout the entire surface of the sample.

As is clear from the results shown in above table, in the conventional processing bath, microorganisms grew to a great extent when the sample was stored for 21-28 days, while in the sample processed in the processing bath of the present invention, the growth of microorganisms was not observed even when the sample was stored for 56 days.

The microorganisms which grew in the experiment were red-purple molds and as the growth of the microorganisms in the comparison cases, gelatin as the protective colloid was attacked to damage the images.

#### EXAMPLE 5

Each of the processing baths W-Z having the following composition and the processing baths A-F shown in Example 1 was subjected to a running test for 56 days at a rate of 5 hours/day while supplying a fresh solution at a rate of 66 ml/0.89 m<sup>2</sup>.

| tb                      | Bath:  |        |       |       |      |
|-------------------------|--------|--------|-------|-------|------|
|                         | W      | X tn Y | Z     |       |      |
| Compound                |        |        |       |       |      |
| Tartaroc                | 10.0 g | 10.0G  | 10.0g | 10.0g |      |
| Acid                    |        |        |       |       |      |
| Zinc                    | 10.0g  | 10.0g  | 10.0g | 10.0g |      |
| Sulfate                 |        |        |       |       |      |
| Sodium                  | 20.0g  | 20.0g  | 20.0g | 20.0g |      |
| Metaborate              |        |        |       |       |      |
| Monomethylol            | 0.2g   |        |       |       |      |
| Hydantoin               |        |        |       |       |      |
| Pentachloro-phenol      |        | 0.5g   |       |       |      |
| Sodium                  |        |        |       |       |      |
| 2-Nitro-1,3-propanediol |        |        | 0.2g  |       |      |
| Pyrogallol-1,3-dimethyl |        |        |       |       | 1.0g |
| Ether                   |        |        |       |       |      |

Water added to make 1 liter in all the cases.

The state of the growth of microorganisms was observed for each processing bath. The results obtained are shown in the following table.

| Bath | Days:  |         |         |         |         |
|------|--------|---------|---------|---------|---------|
|      | 7 days | 14 days | 21 days | 28 days | 56 days |
| A    | 230    | 30 +    | 30 ++   | ∞       | 30 ++   |
| B    | 0      | 0       | 0       | 0       | 0       |
| C    | 0      | ++      |         | +++     | ++      |
| D    | 0      | +       | ++      | +++     | +++     |
| E    | 0      | 0       | 0       | 0       | 0       |
| F    | 0      | 0       | 0       | 0       | 0       |
| W    | 0      | +       | ++tn    | ++      | +++     |
| Y    | 0      | 0       | 30      | ++      | +++     |
| Z    | 0      | 0       | 0       | 0       | 0       |

In the above table, (0) means that the growth of microorganisms was not observed; (+) means the microorganisms grew slightly; (++) means the microorganisms grew considerably; and (+++) means the microorganisms grew throughout the entire surface of the sample.

As is clear from the results shown in the above table, the growth of microorganisms was observed in the conventional processing bath A after running the test for 1 week and also the growth of microorganisms was observed in the conventional processing baths C, D, W,

and X after running the test for 2 weeks. Because the growth of microorganisms was observed in the conventional processing bath Y after running the test for three weeks, the processing bath demonstrated some effect for preventing the growth of microorganisms but such an effect was insufficient in the running test of a long period of time. On the other hand, no growth of microorganisms was observed in the processing bath of this invention even after running the test for 56 days.

The microorganisms which grew in the conventional processing baths during the experiments were black colloidal substances emitting a bitter putrid smell.

The same results were obtained for the processing baths G, N, Q, and R of the present invention. Furthermore, when the compound in the present invention was incorporated in the developing solution, the fixing solution, the bleaching solution or the blixing solution referred to above, the growth of microorganisms in the processing solution was considerably prevented.

While the invention has been described in detail and with reference to specific embodiments thereof, it will be apparent that various changes and modifications can be made therein without departing from the spirit and scope thereof.

What is claimed is:

1. A method of stabilizing a silver halide color photographic material in the development of said material forming color images comprising processing said material in a color photographic processing composition containing pyrogallol-1,3-dimethyl ether.

2. The method of stabilizing the color photographic material according to claim 1, wherein said pyrogallol-1,3-dimethyl ether in said processing composition ranges from about 0.1 to 10g/liter.

3. The method of stabilizing the color photographic material according to claim 1, wherein said color photographic processing composition is an aqueous stabilization solution.

4. The method of stabilizing the color photographic material of claim 1, wherein said processing is after said forming of said color images.

5. The method of stabilizing the color photographic material of claim 1, wherein said processing is prior to said forming of said color images.

6. The method of stabilizing the color photographic material according to claim 1, wherein said color photographic processing composition additionally contains diethylene glycol, polyethylene glycol or mixtures thereof.

7. A stabilized silver halide color photographic material processed in a processing composition according to the method of claim 1.

8. A silver halide color photographic processing and stabilizing composition containing pyrogallol-1,3-dimethyl ether and at least one member selected from the group consisting of urea, a water-soluble derivative of urea, guanidine, a water-solution derivative of guanidine, dihydroxybenzene, a derivative of dihydroxybenzene, trihydroxybenzene, a derivative of trihydroxybenzene, and a phenolic compound.

\* \* \* \* \*